

[54] **PROCESS OF MANUFACTURING FINE POWDERS OF METAL HALIDE**

[75] Inventors: **Norio Kanetake, Tokyo; Ikuo Maruyama, Kawasaki; Katsuyuki Morita, Fujisawa, all of Japan**

[73] Assignee: **Kabushiki Kaisha Kito, Kanagawa-ken, Japan**

[22] Filed: **May 19, 1971**

[21] Appl. No.: **144,809**

[30] **Foreign Application Priority Data**

May 21, 1970 Japan..... 45/43127  
Oct. 10, 1970 Japan..... 45/93630  
Oct. 10, 1970 Japan..... 45/93631

[52] **U.S. Cl. .... 148/6.24, 117/107.2 R, 117/71 M, 117/107.2 P, 148/6.3, 148/6.11, 423/561, 29/195**

[51] **Int. Cl. .... C23f 7/24**

[58] **Field of Search..... 148/6.24, 6.3; 204/37 R; 117/107.2 P, 107.2 R, 71 M; 423/561; 29/195**

[56] **References Cited**

**UNITED STATES PATENTS**

|           |         |                    |            |
|-----------|---------|--------------------|------------|
| 2,399,019 | 4/1946  | Grinter .....      | 148/6.24 X |
| 2,671,739 | 3/1954  | Länder .....       | 117/106 R  |
| 2,903,384 | 9/1959  | Grass et al. ....  | 148/6.24   |
| 2,263,905 | 11/1941 | Snow .....         | 148/6.24   |
| 2,639,245 | 5/1953  | Baxter.....        | 148/6.24   |
| 2,588,234 | 3/1952  | Henricks.....      | 148/6.24 X |
| 3,127,346 | 3/1964  | Oliver et al. .... | 148/6.24 X |

**Primary Examiner—Ralph S. Kendall**

**Attorney—John J. McGlew and Alfred E. Page**

[57] **ABSTRACT**

An improved process for protecting metals against corrosion and wear comprises depositing a coating of metal halide or sulfide as a fine powder in a dry system to the metal surface to be protected in a dry system substantially free from moisture and carbon. Also, provision is made for making finely divided, dry metal halides and sulfides, such as chromium chloride and chromium sulfide which are suitable for use as lubricants and wear-proof and corrosion-proof agents for metals.

**8 Claims, 8 Drawing Figures**



PATENTED OCT 30 1973

3,769,098

SHEET 1 OF 3

FIG. 1



FIG. 2



INVENTORS  
NORIO KANETAKE  
BY IKUO MARUYAMA  
KATSUYUKI MORITA  
John J. McGlew  
ATTY.

FIG. 3



FIG. 4



FIG. 5



FIG. 6



INVENTORS  
 NORIO KANETAKE  
 IKUO MARUYAMA  
 BY KATSUYUKI MORITA  
*John J. McGlew*  
 atty.

FIG. 7



FIG. 8



## INVENTORS

NORIO KANETAKE  
IKUO MARUYAMA  
BY KATSUYUKI MORITA

*John J. McGlew  
atty.*

**PROCESS OF MANUFACTURING FINE POWDERS  
OF METAL HALIDE**

This invention relates to an improvement in the process of manufacturing fine powders of metal halide.

Chromium chloride, chromium bromide, aluminium chloride, aluminium bromide, etc. are used for surface treatment such as in chromium cementation; aluminium cementation; chromium evaporation and aluminium evaporation of steel products. These metal halides are also used as the materials for the manufacture of pure metallic powders of these metals.

For the manufacture of these metal halides, a wet system has generally been adopted so far. However, in the case of the wet system, since a hydrate is liable to be produced, it is difficult to obtain an anhydrous metal halide. Also, since a metal halide containing moisture produces oxide upon the surface treatment of steel products, such a metal halide containing moisture cannot be employed for surface treatment of steel.

On the other hand, in the case of a dry system, for instance, chromium chloride can be manufactured by the reaction of hydrogen chloride gas with chromium as described below:



However, chromium chloride, when produced, assumes the shape of a needle or mass, and in order to make such chromium chloride into fine powders, these materials must be mechanically pulverized because chromium chloride has the properties of deliquescence. However, such pulverization is industrially difficult in operation and the obtaining of yields of chromium chloride powder in abundance is impossible.

This invention aims at providing a process of manufacturing the fine powders of anhydrous metal halide industrially and easily. The invention also relates to a process of manufacturing fine powders of metal halide, which comprises evaporating a metal halide by heating to its fusing point or higher an occluded body of the metal halide in a receptacle in a heating chamber, and then drying an inert gas at a low temperature; the inert gas is supplied in the heating chamber and the metal halide is evaporated and quenched, whereby the halide is made into fine powders and the fine powders of that metal halide are emitted from the heating chamber in a dry state.

Further, this invention also relates to a process of manufacturing a fine powder-like lubricant consisting of chromium sulfide. The invention further relates to a process of manufacturing a fine powder-like lubricant, which comprises evaporating chromium halide by heating to its fusing point or higher an occluded body of chromium halide in a receptacle in the heating chamber, and then supplying a dried mixed gas consisting of inert gas and hydrogen sulfide gas at low temperature to the heating chamber; by the reaction of evaporated chromium halide with hydrogen sulfide gas, chromium sulfide is produced and chromium sulfide is quenched, whereby the chromium sulfide is made into fine powders, and then the fine powders of chromium sulfide are emitted to the heating chamber in a dry state.

Furthermore, this invention relates to a process of wear-proof and corrosion-proof treatment by which both improved wear-proof and corrosion-proof metal products, such as steel products, or non-ferrous metals can be obtained.

The process of improving wear-proof metal products, such as, for instance, gears made of carbon steel, so far has been a known chemical process. For example carburizing, hardening or nitriding, sulphurizing is known and a physical process such as induction hardening is also known. On the other hand, other means for obtaining wear-proof liquid-like lubricant or powder-like lubricant are also known.

However, in the case of the improvement in wear-proofing mentioned above, there was a defect that the simultaneous improvement of wear-proofing and corrosion-proofing is impossible.

This invention aims at providing a process of wear-proofing and corrosion-proofing treatment by which both wear-proof and corrosion-proof metals can be improved. The invention relates to a process of wear-proof and corrosion-proof treatment of metal products, which comprises forming a chromium zone beforehand on the surface of metal products, such as iron and steel, or non-ferrous metals; and reacting the chromium with nitrogen, whereby chromium nitride is produced on the surface of the metal products.

This invention will be better understood with reference to the examples shown in the drawing.

FIG. 1 is a perspective view showing a hollow cylindrical metal halide occluded body;

FIG. 2 is a longitudinal sectional side view showing manufacture of metal halide according to this invention;

FIG. 3 is a view showing a longitudinal temperature distribution of a retort;

FIG. 4 is a view showing a temperature distribution of a section of the retort;

FIG. 5 is a longitudinal sectional side view showing the reaction of sulphur with metal products cemented with chromium or plated with chromium, performed in salt;

FIG. 6 is an enlarged schematic view showing a section through the surface of the metal products obtained according to the invention after a wear-proof and a corrosion-proof treatment was performed;

FIG. 7 is a diagram graphically showing a result of a wear-proof and corrosion-proof test; and

FIG. 8 is a longitudinal sectional side view showing apparatus in which treatment by the reaction of chromium with sulphur is performed in the mixed gas atmosphere.

First, as shown in FIG. 1, a metal halide occluded body 1 formed in the shape of a hollow cylinder is manufactured from a porous body out of the same kind of metal (chromium in case of chromium halide); in this process, metal halide (for instance, chromium halide) is occluded in such a way that it does not contain carbon and oxidizing agent, such as moisture, and hydroxyl; the resulting metal halide occluded body is placed in a retort 2 (shown in FIG. 2).

Next, as seen in FIG. 2, inert gas such as argon or nitrogen gas is supplied from a feed pipe 4 with a valve 3 connected to one end of the retort 2 and the air in the retort is replaced by the inert gas. Then, heating was carried out from the outer periphery of the retort 2 by means of an electric furnace 5 and thus a stream of said metal halide is generated in the retort. Then, a dried inert gas at low temperature is blown into the retort from the feed pipe 4 at one end of the retort 2. Evaporated metal halide in said retort is quenched with the inert gas (in order to perform a further quenching, the

retort 2 is sometimes cooled by means of a cooling means 5') whereby the evaporated metal halide is made into fine powders and the stream of fine powders of this metal halide in inert gas is withdrawn into a storage tank 8 which is maintained in dried condition from the other end of the retort 2 through a feed pipe 7 with a valve 6 by means of which said inert gas stream is admitted.

At the upper part of the storage tank 8, there is a filter 9 for venting the inert gas and preventing the escape of fine powders of the metal halide; at the lower part of the storage tank 8, there is an exhaust port 10 having a valve 10.

FIG. 3 shows a longitudinal temperature distribution curve for the retort 2, in which:  $\theta_1$  indicates a temperature lower than the fusing point of metal halide,  $\theta_2$  indicates a temperature at the heating zone of the retort and this temperature is higher than the fusing point of metal halide,  $\theta_3$  indicates a temperature lower than  $\theta_2$ , and this temperature is lower than the fusing point of metal halide; in particular, there is no need of heating or heat retaining, but rather a remarkably lower temperature (about 600°–900°C) than  $\theta_2$  is suitable for making evaporated metal halide into fine powders.

As to the temperature distribution in the retort, shown in section in FIG. 3, it is necessary to maintain the temperature where inert gas flows lower than the temperature at the point where the metal halide occluded body is heated and it is also necessary to make the former temperature lower than the fusing point of metal halide in order to solidify the evaporated metal halide.

Further, in carrying out this invention, the heating chamber, (for instance, the retort) may be longitudinally or obliquely directed, instead of laterally, as shown in the drawing; or its section may be circular, oval, square or other shapes.

Instead of the electric furnace, a gas furnace or a heavy oil furnace may be used as the heating furnace. Further, any outer-heat system or inner-heat system or both inner- and outer-heat system may be adopted as heating chamber.

The invention is illustrated further below with reference to the embodiments of this invention described herein:

The retort 2 in the apparatus shown in FIGS. 2 and 3 having a cylindrical retort is made of stainless SUS 27 of 5cm in diameter and 2m in length. Into this retort is introduced 100 kg of a chromium chloride halide occluded body consisting of chromium chloride ( $\text{CrCl}_2$ ) about 20 – 60%, iron (Fe) 0.5% or less, aluminium oxide ( $\text{Al}_2\text{O}_3$ ) or silicon oxide ( $\text{SiO}_2$ ) about 5–30 percent and remaining amount of chromium. Then, argon is supplied to the retort from the feed pipe 5 thereby expelling the air in the retort and then the retort is heated by means of the electric furnace 5. As the heating condition  $\theta_1$  shown in FIG. 3 is determined at 20°–100°C,  $\theta_2$  at 1,000°C, (higher than 815°C), the fusing point of chromium chloride,  $\theta_3$  at 200°–400°C (in order to perform further cooling, a cooling means 5' is employed and  $\theta_3$  is sometimes determined at 30°–100°C.) 20 l/min. of argon gas is supplied from the feed pipe 4 and a temperature distribution of the section of the retort inside is made as shown in FIG. 4. The chromium chloride which is evaporated in the retort is quenched with argon gas to make into fine powders, and thus the fine powders of anhydrous chromium

chloride of  $0.5\text{--}1\mu$  in diameter and of 99.9 percent in high purity was obtained.

This invention is carried out as described above, namely, the occluded metal halide body is placed in the heating chamber and is heated to its fusing point or higher; the metal halide is evaporated, dispersed and then a dried inert gas at low temperature is introduced into the heating chamber. The metal halide which is evaporated and dispersed is quenched and solidified; therefore, the fine powders of metal halide thus obtained can be easily and continuously produced in abundance by skillfully utilizing the evaporating and dispersing action, as well as the cooling and solidifying action. Further, the cooling takes place with the inert gas, so that oxidation can be prevented and fine powders of anhydrous metal halide of high purity can be manufactured.

Further, instead of the inert gas used in the above-mentioned illustrative embodiment, a dried mixed gas at low temperature consisting of 80 percent inert gas (for example, argon or nitrogen gas) and 20 percent hydrogen sulfide gas, is used; the mixed gas is introduced in the heating chamber from the feed pipe 4 at one end of the retort 2 and chromium sulfide is produced by the reaction of chromium halide which is evaporated in the retort with oxygen sulfide gas and chromium sulfide is quenched; (in order to perform a further quenching, the retort 2 is sometimes cooled by means of the cooling means 5'); in this manner, chromium sulfide is made into fine powders. Further, it is remarked that the fine powders of this chromium sulfide are stored in the storage tank 8 which is maintained in a drying condition. The chromium sulfide is introduced from the other end of the retort 2 through the feed pipe 7 with the valve 6 by means of said gas blown in. In this case, therefore, chromium sulfide suitable as a lubricant can easily and continuously be produced in abundance by skillfully utilizing the reaction of the chromium halide evaporated and dispersed with the hydrogen sulfide gas evaporated and dispersed and the quenching and solidifying action by means of feed gas.

Explanation of the invention is made below with reference to FIGS. 5 to 8 in other illustrative embodiments and examples.

#### EXAMPLE 1

A carbon steel gear is provided having a chemical composition of C: 0.42%, Mn: 0.68%, Si: 0.21%, P: 0.015% and S: 0.026%. This gear is placed with a chromium chloride generating substance in an atmospheric furnace in which the atmosphere can be controlled from the outside. After the air in the furnace is eliminated, a temperature in the furnace is maintained at 1,000°C for 5 hours. Chromium is thus cemented on the surface of the gear and thereafter the gear is at once put in oil and quenched so that hardening of the gear takes place.

Next, as shown in FIG. 5, in the case 12 provided in the electric furnace 11, the quenched gears 14 are immersed for 1 hour heated at 200°C in a mixed salt 13 of sodium sulfate (85%) and potash alum (15%). The gears are then air-cooled. As shown in FIG. 6, a matrix 15 of tempered martensite, a chromium cementation zone 16 ( $15\mu$  in average thickness), a chromium zone 17 ( $20\mu$  in average thickness) and a chromium sulfide zone 18 ( $2\mu$  in average thickness) are produced in

turn. The structure of the matrix is illustrated in section by FIG. 6. A wear-proof and corrosion-proof treated gear of HRC49 in surface hardness was thus obtained.

In similar fashion, another gas consisting of carbon steel of the same composition as described above is heated at 1,000° C, and after oil hardening, quenching is performed at 200° C and thus a heat-treated gear of HRC49 in hardness was also obtained.

The two kinds of gears obtained, as described above, are engaged with gears of the same kind respectively without feed oil and are rotated. Then, a wear loss (decreased amount of tooth thickness) of tooth in pitch circle was measured. The test results showed that merely heat-treated gears are inferior in wear resistance, as indicated by line A of FIG. 7, and such a gear has no corrosion resistance. However, a wear- and corrosion-resistant treated gear according to this invention is remarkably excellent in wear resistance, as indicated by line B of FIG. 7 and also has corrosion resistance.

#### EXAMPLE 2

Chromium cementation gears 14 which are made of carbon steel obtained with the same composition as that of Example 1 are placed in case 12 of electric furnace 11 as shown in FIG. 8. A mixed gas of 70% argon and 30% H<sub>2</sub>S is supplied from gas feed port 21 in lid 20 on which fan 19 is mounted. The air in case 12 is vented from a port hole 22. Thereafter, the gears were taken out after heating at 600° C for 1 hour.

In this example, too, a chromium sulfide zone is formed on the surface of the chromium zone on the gear and the same wear-resistance and corrosion-resistance as in the case of Example 1 was obtained.

#### EXAMPLE 3

After a shaft made of brass is plated (5μ in thickness) with chromium, this shaft is reacted with sulfur in mixed salt as shown in FIG. 1 and thus chromium sulfide (1μ in thickness) was produced on the surface.

When this shaft was inserted in the hole of a bearing and was slided reciprocatingly, wear loss was lowered to 1/5 as compared with a shaft made of brass which was not so treated.

Since this invention is constituted as described hereinabove, it has been found that the chromium sulfide has a lubricating property, namely, a wear-resistance is produced on the surface of the chromium zone having corrosion resistance by merely performing a treatment

such as the reaction of the chromium zone in sulfide after the chromium zone was formed on the surface of metal products merely by chromium cementation or chromium plating. In this manner, both wear-resistance and corrosion resistance of the gears can be improved.

We claim:

1. A process for treatment of metal products to protect the same against wear and corrosion which comprises (1) heating said metal products in presence of a chromium halide in absence of oxygen, whereby chromium is diffused into said metal products forming a chromium zone on the surface thereof (2) reacting the chromium in the zone where the chromium is diffused into the metal products with a sulfur compound to form chromium sulfide on the surface of said metal products, and (3) recovering the metal products protected against wear and corrosion.

2. A process for treatment of metal products, according to claim 1, wherein said metal products comprise ferrous metal.

3. A process for treatment of metal products, according to claim 2, wherein said ferrous metals comprise steel gears.

4. A process for treatment of metal products, according to claim 3, wherein said steel gears are treated with a fine powder deposit of chromium halide in a dry atmosphere and thereafter said chromium coating on the gear is converted to chromium sulfide by reaction with a sulfur compound to yield a steel gear with improved resistance to corrosion and wear.

5. A process for treatment of metal products, according to claim 4, wherein said chromium halide is chromium chloride and said sulfur containing composition is the mixed salt sodium sulfate and potash alum.

6. A process for treatment of metal products, according to claim 1, wherein said metal products are made of non-ferrous metal.

7. A process for treatment of metal products, according to claim 1, wherein said chromium zone is formed in a furnace at about 1,000° C for about 5 hours.

8. A process for treatment of metal products, according to claim 7, wherein the metal products, after treatment with chromium halide in the furnace, are immersed in a bath of mixed salt of potash alum and sodium sulfate at 200° C for 1 hour and thereafter removed from said bath, cooled and recovered.

\* \* \* \* \*